# EUROPEAN PATENT SPECIFICATION

(11) **EP 1 382 703 B1**
(45) Date of publication and mention of the grant of the patent: **26.12.2007**
(21) Application number: 03015517.0
(22) Date of filing: 09.07.2003
(51) Int. Cl.: C22C 38/04, C22C 38/00, C22C 38/12

(54) **Steel pipe having low yield ratio**
Stahlrohr mit einem niedrigem Streckgrenze/Zugfestigkeit-Verhältnis
Tube en acier à bas rapport de la limite d'élasticité à la résistance à la rupture

(30) Priority: 10.07.2002 JP 2002200797
(43) Date of publication of application: 21.01.2004
(73) Proprietor: Nippon Steel Corporation, Tokyo 100-8071 (JP)
(72) Inventor: Ohgami, Masahiro, Nippon Steel Corp. Yawata Works, Kitakyushu-shi, Fukuoka 804-8501 (JP); Fujii, Toshio, Nippon Steel Corp. Hikari Works, Hikari-shi, Yamaguchi 743-8510 (JP); Ogata, Toshiyuki, Nippon Steel Corp. Hikari Works, Hikari-shi, Yamaguchi 743-8510 (JP); Mimura, Hiroyuki, Nippon Steel Corp. Hikari Works, Hikari-shi, Yamaguchi 743-8510 (JP)
(74) Representative: Vossius & Partner

(56) References cited:
- EP-A- 0 757 113
- EP-A- 0 885 978
- WO-A-01/62998
- WO-A-02/40731
- US-A- 3 704 180
- US-A- 4 219 371
- PATENT ABSTRACTS OF JAPAN vol. 1999, no. 14, 22 December 1999 (1999-12-22) -& JP 11 256268 A (NISSHIN STEEL CO LTD), 21 September 1999 (1999-09-21)
- PATENT ABSTRACTS OF JAPAN vol. 1999, no. 01, 29 January 1999 (1999-01-29) -& JP 10 265844 A (SUMITOMO METAL IND LTD), 6 October 1998 (1998-10-06)
- PATENT ABSTRACTS OF JAPAN vol. 1998, no. 05, 30 April 1998 (1998-04-30) & JP 10 017980 A (SUMITOMO METAL IND LTD), 20 January 1998 (1998-01-20)
- PATENT ABSTRACTS OF JAPAN vol. 2000, no. 05, 14 September 2000 (2000-09-14) & JP 2000 054061 A (NIPPON STEEL CORP), 22 February 2000 (2000-02-22)
- EDITED BY CLYDE L. BROWN: "Impurities in Engineering Materials" 1999, MARCEL DEKKER, INC , USA , XP002268595 * page 63 *

## Description

The present invention relates to a steel pipe having a low yield ratio.

It has been clarified recently that it is effective to use a steel material having a low yield ratio, as a structural member, to enhance the earthquake resistance of a building. In that sense, a steel pipe for a building is also required to have a low yield ratio. This is because it is estimated that if the yield ratio of a steel pipe for a building is lower, the steel pipe will seldom rupture, even though it yields, and therefore the structure is less likely to be destroyed.

In the case of a line pipe, highly reliable impact resistance and earthquake resistance are required of a line pipe to avoid the leakage of a transported material such as petroleum or the bursting of the line pipe. In that sense, it is effective to use a steel pipe having a low yield ratio as a line pipe for.greater safety.

In the meantime, with regard to a welded steel pipe, as a welded steel pipe undergoes the influence of cold-working such as bending, pipe expansion, drawing and so on during pipe production, a welded steel pipe having the same low yield ratio as a steel sheet used as the mother material of the steel pipe cannot be obtained, in many cases. Therefore, to obtain a steel pipe having a low yield ratio, it is necessary to sufficiently lower the yield ratio of a steel sheet before it is used in pipe production.

In JP-A-10-17980, an invention is disclosed wherein, in the event of producing a welded steel pipe having a low yield ratio, a steel containing 1 to 3% Cr as an essential component is used as the base steel and the structure of the steel is composed of a composite structure containing a soft ferrite phase and a hard bainite or martensite phase in a manner that is already known.

In JP-A-2000-54061, it is described that a steel material and a steel pipe made of the steel material, that have a low yield ratio at the ordinary temperature and are excellent in strength at a high temperature, can be obtained by controlling the C contained in the steel material to not more than 0.03%, preferably not more than 0.015%, making Nb exist in the state of solid solution and, further, properly controlling the microstructure of the steel material.

In JP-A-2000-239972, it is described that a steel material and a steel pipe made of the steel material, that have a low yield ratio at the ordinary temperature and are excellent in strength at a high temperature, can be obtained by controlling the C contained in the steel material to not more than 0.02%, preferably not more than 0.015%, and adding Nb and Sn abundantly.

The invention disclosed in the aforementioned JP-A-10-17980 requires Cr of not less than 1% as an essential component in order to secure a low yield ratio and a high strength simultaneously by forming a hard phase composed of a bainite phase or a martensite phase. However, the invention cannot provide a low cost steel pipe having a low yield ratio because Cr alloy is expensive. In addition, Cr tends to form oxides during welding and when Cr oxides remain at a weld-butting portion, the quality of a weld deteriorates.

In the inventions disclosed in the aforementioned JP-A-2000-54061 and 2000-239972, a low yield ratio is secured by limiting the upper limit of C to not more than 0.03% and 0.02% respectively, preferably not more than 0.015%, and, by so doing, reducing the amount of solute C at the ordinary temperature. However, in such cases of reducing the C amount as described above, a high tensile strength is seldom obtained in a tensile test at the ordinary temperature.

JP-A-11-256268 discloses a steel plate excellent in local ductility and heat treatability comprising, by mass, C: 0.15 to 0.40%, Si ≤ 0.10%, Mn: 0.3 to 0.8%, P ≤ 0.02%, S ≤ 0.01%, Ti: 0.01 to 0.05%, B: 0.0005 to 0.0050%, N ≤ 0.01 %, T.A1: 0.02 to 0.10%, Cr: 0 to 0.6%, and the balance with Fe and unavoidable impurities, wherein carbides are dispersed in ferrite in such a manner that the carbide spheroidizing ratio is 90% or more and the average carbide grain size is controlled to 0.4 to 10 µm.

The object of the present invention is, by solving the above problems, to provide a steel pipe having a low yield ratio. The object can be achieved by the features specified in the claims.

The feature common to the whole present invention is that the microstructure of a steel pipe is composed of a structure containing ferrite and the average size of the ferrite grains is not smaller than 20 µm. As a yield stress is proportioned to (grain size)^{-1/2} according to Hall-Petch's Law, a yield stress and a yield ratio increase as a grain size decreases. In contrast with this, a yield stress and a yield ratio decrease as a grain size increases. The present invention, based on the above fact, has made it clear that, when the average size of ferrite grains contained in a microstructure is not smaller than 20 µm, a yield stress lowers and as a result a low yield ratio can be obtained even with a steel pipe after subjected to pipe production processes. An average size of ferrite grains is preferably not smaller than 30 µm, still preferably not smaller than 40 µm.

The average size of grains including ferrite grains is measured in accordance with the method described in the Appendix 1 of JIS G 0552. In the case of martensite or bainite, the size of prior austenite grains is measured and it is recommended to conform to the Appendix 3 of JIS G 0551.

It is preferable that the content rate of ferrite in a microstructure is in the range from 70 to 98%. The reason is that, when the content rate of ferrite is less than 70%, a yield stress cannot be lowered sufficiently even with a ferrite grain size increased and therefore a low yield ratio cannot be obtained. However, when the content rate of ferrite exceeds 98%, the tensile strength of a steel lowers and therefore a low yield ratio cannot be obtained likewise. It is still preferable that the content rate of ferrite is in the range from 75 to 95%.

Here, the content rate of ferrite in a microstructure in the present invention means a volume traction of ferrite in the microstructure.

In conventional hot rolling of a steel sheet used for producing a steel pipe having a low yield ratio, the steel sheet has been rolled in the temperature range from a temperature of the γ phase region to a lower side temperature of the two-phase region after it is heated to a temperature of the γ phase region. Therefore, it has been impossible to make the average ferrite grain size not smaller than 20 µm. The present invention has made it possible to: finish rolling in the temperature range from a temperature of the γ phase region to a higher side temperature of the two-phase region after a steel is heated to a temperature of the γ phase region; thus suppressing the fractionization of grains; and, as a result, produce a steel having an average ferrite grain size of not smaller than 20 µm. It is possible to make the average ferrite grain size not smaller than 20 µm by controlling a cooling rate to not more than 10°C/sec. up to the temperature of the Ar₁ point + 50°C after the end of hot rolling.

Furthermore, it is possible to make the average ferrite grain size not smaller than 30 or even 40 µm by controlling a temperature at the end of hot rolling, a cooling rate after the end of hot rolling, and so on.

The present invention is so constituted of that a microstructure is composed of ferrite and pearlite.

In the invention, a microstructure is composed of ferrite and pearlite. That means that the microstructure is a structure that contains ferrite as an essential phase and additionally pearlite. As a result of composing such a structure, a steel pipe having a low yield ratio and a tensile strength of 500 to 600 MPa can be produced.

The reasons for limiting the chemical components in the invention are explained hereunder.

C is an element that precipitates as solid solution or carbides in a matrix and enhances the strength of a steel. Further, C precipitates also as the second phase composed of cementite and pearlite. Therefore, in the event of forming a hot-rolled steel sheet into a steel pipe by cold forming, C suppresses the increase of a yield stress or proof stress, enhances tensile strength and uniform elongation, and resultantly contributes to the lowering of a yield ratio. C is required to be contained at not less than 0.01%, preferably not less than 0.04%, for securing the effect of cementite, etc. precipitating as the second phase on the lowering of a yield ratio. However, when C is contained in excess of 0.20%, the effect of lowering a yield ratio and weldability deteriorate. For these reasons, a C content is limited to the range from 0.01 to 0.20%.

Si functions as a deoxidizer and enhances the strength of a steel by dissolving in a matrix. The effect appears with a Si content of not less than 0.05%. On the other hand, when Si exceeds 1.0%, the effect of lowering a yield ratio deteriorates. For these reasons, the Si content is limited to the range from 0.05 to 1.0%.

Mn is an element that enhances the strength of a steel and accelerates the precipitation of cementite or pearlite composing the second phase. The effects appear with a Mn content of not less than 0.1%. On the other hand, when Mn is contained in excess of 2.0%, the effect of lowering a yield ratio deteriorates. For these reasons, the Mn content is limited to the range from 0.1 to 2.0%. Here, from the viewpoint of strength and toughness, it is preferable that the Mn content is in the range from 0.3 to 1.5%.

Al is used as a deoxidizer but the amount of Al significantly influences a grain size and mechanical properties. An Al content of less than 0.001% is insufficient as a deoxidizer. On the other hand, when Al exceeds 0.05%, oxides containing Al increase in a steel and deteriorate toughness. For these reasons, the Al content is limited to the range from 0.001 to 0.05%.

A microstructure composed of ferrite and pearlite according to the invention is obtained by: finishing rolling in the temperature range from a temperature of the γ phase region to a higher side temperature of the γ-α two-phase region after a steel is heated to a temperature of the γ phase region; thereafter cooling the steel at a cooling rate of not more than 10°C/sec. up to the temperature of the Ar₁ point + 50°C; and successively cooling the steel at a cooling rate of not less than 3°C/sec. in the temperature range not higher than the temperature of the Ar₁ point + 50°C.

In the invention, it is preferable that a microstructure further contains spheroidized pearlite. The reason is that, when such a structure is contained, the increase of a yield ratio can be suppressed in the event of forming a steel sheet into a steel pipe. In addition, spheroidized pearlite has the effect of improving uniform elongation.

It can be determined whether pearlite is spheroidized or not by defining pearlite as it is spheroidized when an aspect ratio between the length and the width of the second phase is not more than 2 in a section parallel with the rolling direction.

The spheroidization of pearlite can be done by: heating a steel material to a temperature in the range of 1,150°C ± 50°C; thereafter finishing the hot rolling of the steel material at a temperature of not lower than the Ar₁ point and thus producing a steel strip about 10 mm in thickness to which strain (dislocation) is introduced; and successively cooling the steel strip at a cooling rate of 3 to 30°C/sec. up to a temperature of not higher than 700°C, then coiling it, and, in the meantime, precipitating pearlite at grain boundaries or on dislocations.

Further, in the invention, the average size of pearlite grains grains is 4 to 23 µm. The reason is that, by so doing, the increase of a yield ratio can be suppressed in the event of forming a steel sheet into a steel pipe.

An average pearlite grain size of 4 to 23 µm can be obtained by controlling the cooling rate to not less than 3°C/sec. in the temperature range not higher than the temperature of the Ar₁ point + 50°C after the end of hot rolling.

Still further, in the invention, it is preferable that a steel pipe contains one or both of 0.01 to 0.5% Nb and 0.001 to 0.01% N. Nb is an element that precipitates as solid solution or carbonitrides in a matrix and enhances strength, and therefore Nb is required to be contained by at least 0.01%. However, even though Nb is excessively added in excess of 0.5%, the effect is saturated and a sufficient strengthening effect is not secured or, instead, precipitates coarsen and toughness deteriorates. For these reasons, a Nb content is limited to the range from 0.01 to 0.5%. N exists as solid solution or nitrides in a matrix. A N content of not less than 0.001% is required for forming nitrides that contribute to the strengthening of a steel. However, when N is added in excess of 0.01%, coarse nitrides tend to form and deteriorate toughness. For these reasons, the N content is limited to the range from 0.001 to 0.01%.

Now the reasons for limiting the preferable chemical components for the invention are explained hereunder.

Ti is an element that has the effect of improving weldability and the effect is recognized with a Ti content of not less than 0.005%. However, when Ti is added in excess of 0.1%, the deterioration of workability and an unnecessary increase of strength are caused by the increase of Ti carbonitrides. For these reasons, the Ti content is limited to the range from 0.005 to 0.1%.

B causes grain boundary strengthening and precipitation strengthening by precipitating in the forms of M₂₃(C, B)₆, etc. and thus increases strength. The effect is low with a B content of less than 0.0001%. On the other hand, when the B content exceeds 0.005%, the effect is saturated, a, coarse B-contained phase tends to form, and enbrittlement is likely to occur. For these reasons, the B content is limited to the range from 0.0001 to 0.005%.

V increases strength as a precipitation-strengthening element. The effect is insufficient with a V content of less than 0.01%. On the other hand, when a V content exceeds 0.5%, not only carbonitrides coarsen but also the increment of yield strength increases. For these reasons, the V content is limited to the range from 0.01 to 0.5%.

Cu is an element that increases strength. When a Cu content is less than 0.01%, the effect is low. On the other hand, when Cu is added in excess of 1%, the increment of yield strength increases. For these reasons, the Cu content is limited to the range from 0.01 to 1%.

Ni is an element that increases strength and also is effective for improving toughness. When a Ni content is less than 0.01%, the effect of improving toughness is low. On the other hand, when Ni is added in excess of 1%, the increment of yield strength increases. For these reasons, the Ni content is limited to the range from 0.01 to 1%.

Cr increases strength as a precipitation-strengthening element. The effect is insufficient with a Cr content of less than 0.01%. On the other hand, when the Cr content exceeds 1%, not only carbonitrides coarsen but also the increment of yield strength increases. For these reasons, the Cr content is limited to the range from 0.01 to 1%.

Mo causes solid solution strengthening and at the same time increases strength. When a Mo content is less than 0.01%, the effect is low. On the other hand, when Mo is added in excess of 1%, the increment of yield strength increases. For these reasons, the Mo content is limited to the range from 0.01 to 1%.

A steel according to the present invention can be provided in the forms of not only a steel pipe produced by cold-forming a hot-rolled steel sheet but also a steel plate and a steel sheet. Further, as an example of a product produced by cold-working a steel according to the present invention, an electric resistance welded steel pipe is nominated. With regard to the effects of the present invention, the effect of lowering a yield ratio is prominent when a low strain pipe forming method is employed.

### EXAMPLE

Steels having the components shown in Table 1 were produced into continuously cast slabs and then the slabs were hot rolled into steel sheets 10 mm in thickness. In the hot-rolling process: the slabs were heated to a temperature of 1,150°C; thereafter the hot rolling was finished at a temperature of 900°C (Ar₁ point + 170°C) and thus strain (dislocation) was introduced; successively the steel sheets were cooled at the cooling rates in the range from 5 to 15°C/sec. up to a temperature of not higher than 700°C; and then the steel sheets were coiled.

The microstructures of the steel sheets are shown in Table 2. The tensile properties of a steel sheet were evaluated by using an as-rolled specimen of the steel sheet to which no working was applied and a specimen thereof to which 5%-prestrain was applied. 5%-prestrain corresponds to the cold-working applied for forming a steel sheet 10 mm in thickness into a steel pipe 200 mm in diameter. In general, prestrain is applied so as to equal the value of t (steel pipe thickness)/D (steel pipe diameter) with respect to a steel pipe to be produced. The prestrain was given by the method wherein a tensile test specimen was pulled with a tensile tester and the pulling was stopped at the time when the strain reached 5%. The tensile properties evaluated were YS (yield strength), TS (tensile strength) and YR (yield ratio). The results of the evaluation are shown in Table 2.

In the cases of the invention examples Symbols A-1 to G-1, the steel components were within the ranges specified in the present invention and any of the average ferrite grain sizes was not smaller than 20 µm. The yield ratios (YRs) of the 5%-prestrain specimens were in the range from 71 to 89%. In the cases of Symbols B-1, D-1 and G-1 wherein pearlite was spheroidized, the YRs of the 5%-prestrain specimens were lower than the other specimens.

In the cases of the comparative examples Symbols H-1 to O-1, any of the steel components deviated from the ranges specified in the present invention. The average ferrite grain sizes were smaller than 20 µm in the cases of Symbols J-1, L-1, M-1 and O-1. These were the examples wherein YRs increased because YSs increased after 5%-prestrain was imposed. There were no cases where pearlite was spheroidized and, in the cases of Symbols H-1 to K-1, M-1 and N-1, the average grain sizes of the pearlite were outside the preferable range of not larger than 20 µm. These were the examples wherein pearlite that composed the second phase grew larger because the cooling rates were less than 3°C/sec. in the temperature range of not higher than Ar₁ point + 50°C after the end of hot rolling. Here, the yield ratios (YRs) of the 5%-prestrain specimens were in the range from 91 to 98%. These were the examples wherein YSs increased and thus YRs increased because the grain sizes of pearlite that composed the second phase were large and therefore the pearlite grains acted as resistance to deformation when 5%-prestrain was imposed.

The present invention makes it possible to: reduce the production cost of a low yield ratio steel pipe by suppressing the Cr content; enhance tensile strength at the ordinary temperature by suppressing the formation of Cr oxides that deteriorate the quality of a weld and raising the upper limit of the C content; and thus obtain, a low yield ratio steel pipe.

## Claims

1. A steel pipe having a low yield ratio, **characterized in that**: the steel pipe contains, in mass, 0.01 to 0.2% C, 0.05 to 1.0% Si, 0.1 to 2.0% Mn, 0.001 to 0.05% Al and optionally one or more selected from 0.01 to 0.5% Nb, 0.001 to 0.01% N, 0.005 to 0.1% Ti, 0.0001 to 0.005% B, 0.01 to 0.5% V, 0.01 to 1% Cu, 0.01 to 1% Ni, 0.01 to 1% Cr and 0.01 to 1% Mo, with the balance consisting of Fe and unavoidable impurities; the microstructure of the steel pipe is composed of ferrite and pearlite; and the average size of the ferrite grains is not smaller than 20 µm; and the average size of the pearlite is 4 to 23 µm.

2. A steel pipe having a low yield ratio according to claim 1, **characterized in that** the microstructure of the steel pipe contains spheroidized pearlite.

3. A steel pipe having a low yield ratio according to claim 2, **characterized in that** the average size of pearlite grains is not larger than 20µm.

## Patentansprüche

1. Stahlrohr mit kleinem Streckgrenzverhältnis,
**dadurch gekennzeichnet, dass** das Stahlrohr in Masse-% enthält:
0,01 bis 0,20% C;
0,05 bis 1,0% Si;
0,1 bis 2,0% Mn;
0,001 bis 0,05% Al; und
optional eines oder mehrere der folgenden Komponenten in den entsprechenden Anteilen:
0,01 bis 0,5% Nb;
0,001 bis 0,01% N;
0,005 bis 0,1% Ti;
0,0001 bis 0,005% B;
0,01 bis 0,5% V;
0,01 bis 1% Cu;
0,01 bis 1% Ni;
0,01 bis 1% Cr; und
0,01 bis 1% Mo;
wobei der Rest aus Fe und unvermeidbaren Verunreinigungen besteht;
wobei die Mikrostruktur des Stahlrohrs aus Ferrit und Perlit besteht, und wobei die mittlere Partikelgröße der Ferritkörner nicht kleiner ist als 20 µm; und
wobei die mittlere Größe des Perlits 4 bis 23 µm beträgt.

2. Stahlrohr nach Anspruch 1, **dadurch gekennzeichnet, dass** die Mikrostruktur des Stahlrohrs körniges Perlit aufweist.

3. Stahlrohr nach Anspruch 2, **dadurch gekennzeichnet, dass** die mittlere Größe der Perlitkörner nicht größer ist als 20 µm.

## Revendications

1. Tube en acier à bas rapport de la limite d'élasticité à la résistance à la rupture, **caractérisé en ce que** : le tube en acier contient, en masse, C à 0,01 à 0,20 %, Si à 0,05 à 1,0 % ; Mn à 0,1 à 2,0 %, Al à 0,001 à 0,05 % et facultativement un ou plusieurs éléments choisis parmi Nb à 0,01 à 0,5 %, N à 0,001 à 0,01 %, Ti à 0,005 à 0,1 %, B à 0,0001 à 0,005 %, V à 0,01 à 0,5 %, Cu à 0,01 à 1 %, Ni à 0,01 à 1 %, Cr à 0,01 à 1 % et Mo à 0,01 à 1 %, le reste consistant en Fe et des impuretés inévitables ; la microstructure du tube en acier est composée de ferrite et de perlite ; et la taille moyenne des grains de ferrite n'est pas inférieure à 20 µm ; et la taille moyenne de la perlite est de 4 à 23 µm.

2. Tube en acier à bas rapport de la limite d'élasticité à la résistance à la rupture selon la revendication 1, **caractérisé en ce que** la microstructure du tube en acier contient de la perlite globulaire.

3. Tube en acier à bas rapport de la limite d'élasticité à la résistance à la rupture selon la revendication 2, **caractérisé en ce que** la taille moyenne des grains de perlite n'est pas supérieure à 20 µm.
